

March 8, 1966

R. G. GUENTER

3,239,583

SMOKELESS POWDER MANUFACTURE

Filed June 8, 1946



FIG.1



FIG.2

RICHARD G. GUENTER  
INVENTOR.

BY

*Ernest G. Peterson*  
AGENT

## 1

3,239,583

**SMOKELESS POWDER MANUFACTURE**  
 Richard G. Guenter, Kenil, N.J., assignor, by mesne assignments, to the United States of America as represented by the Secretary of the Army  
 Filed June 8, 1946, Ser. No. 675,435  
 10 Claims. (Cl. 264—3)

This invention relates to the manufacture of cast propellents and, more particularly, to a large cast propellant and method of making same whereby faultily prepared castings are detected and eliminated.

In the casting of large smokeless powder propellents by the method involving curing a mixture of casting powder, burning rate control powder, and nonvolatile plasticizers at elevated temperatures, it is essential that all components be uniformly distributed throughout to form a homogeneous casting. Local concentration of nonvolatile plasticizer, casting powder, or burning rate control powder, as well as entrapped air cause fluctuations during burning and can lead to uncontrolled fast burning with high pressure development and even rupture of the combustion chamber walls of jet-controlled devices in which such powders may be used.

Uniform distribution is difficult to obtain, particularly when the burning rate control powder is in the form of granules comparable in size to the casting powder granules. Thus, when the powders are blended and added to the casting container or mold, the denser burning rate control particles tend to segregate. This tendency is increased when the blended powder granules and the liquid plasticizers are added to the mold in successive increments and agitated in accordance with methods heretofore used.

The tendency to segregation may be minimized by employing the improved casting methods disclosed in the copending application of Donald L. Black, Ser. No. 675,436, filed June 8, 1946, now Patent No. 3,205,286, which involves placing the blended powder in a mold, placing a weight on top of the powder and introducing the liquid plasticizers through an opening in the bottom of the mold. Nevertheless, it is possible that through careless manipulation or for other reasons, segregation may sometimes occur, thus resulting in a faulty casting which should be eliminated.

Although it is important that faulty castings be detected and eliminated, this has not been easily possible heretofore. Visual methods have been generally unsatisfactory due to the difficulty of distinguishing the individual components. Thus, where the burning rate control powder is in the form of granules, the granules of casting powder and of burning rate control powder are all about the same size, shape, and color, making it difficult to pick up nonuniformities. Again, where the burning rate control powder is in the form of filaments or strands, flaws in the finished casting, such as irregular placement of the filaments or introduction of an improper number of filaments, are not easily detectable.

X-rays have been used to some extent to detect faulty castings but do not give satisfactory results in all cases. Furthermore, the use of X-rays is tedious, time consuming, and expensive, and hence is not desirable for these reasons.

Now, in accordance with the present invention, it has been found that faulty cast propellents may be detected and eliminated by a method involving forming the powder components with distinctly different colors. Furthermore, it has been found that the novel cast propellents of this invention have properties such that the homogeneity of the casting may be determined by visual inspection.

In general, the powder components to be utilized com-

## 2

prising a casting powder, a burning rate control powder, and a casting solvent, will have incorporated therewith materials which will impart to the components distinctive colors. Alternatively, the powder components may be coated with or otherwise treated by suitable materials to impart the desired distinctive colors. The casting powder and burning rate control powder are then mixed, added to a transparent casting container, and the casting solvent introduced through an opening in the bottom. The container contents are then cured at elevated temperatures to form the cast propellant.

When the mixture of casting powder and burning rate control powder is added to the casting container, the different colored granules of each form a color pattern which gives a visual indication of the uniformity of distribution of the granules. Thus, a local concentration of granules of one color is readily picked up and indicates that the distribution is faulty. The faulty mixture may thereupon be eliminated at this stage of the process, thus saving the additional time, expense, and labor necessary to complete the casting of the charge. Visual indication is also possible at subsequent points in the operation, such as after the casting solvent is added, and after the charge is cast. In each case, the color pattern indicates the uniformity of distribution of the powder components in the casting and facilitates detection and elimination of faulty castings. When rate control powder in the form of strands of distinctive color is utilized, examination of the ends of the casting reveals omission or nonuniform spacing of the strands.

The cast propellant in accordance with this invention is illustrated in the accompanying drawing in which:

FIG. 1 is a view showing a cast propellant charge having the powder components distributed uniformly throughout, and

FIG. 2 is a view showing a faulty cast propellant charge having local concentrations of rate control granules.

In a homogeneous casting as shown in FIG. 1, the different colored particles blend into a harmonious pattern giving the effect of uniformity. Local concentrations of one material emphasize the particular color of that material in the locale of the concentration and are easily detected as shown in FIG. 2.

In accordance with the invention and to illustrate more particularly the improved product and method of producing it, the following example is given:

*Example*

Twenty-one castings were prepared using powder components as follows:

|                           | Casting Powder, percent | Burning Rate Control Powder, percent | Casting Solvent, percent |
|---------------------------|-------------------------|--------------------------------------|--------------------------|
| Nitrocellulose (13.15% N) | 73.5                    | 25.00                                |                          |
| Nitroglycerin             | 20.0                    | 6.66                                 | 74.0                     |
| Carbazole                 | 1.5                     | 1.05                                 | 0.5                      |
| Potassium perchlorate     |                         | 56.00                                |                          |
| Carbon black              |                         | 9.00                                 |                          |
| Diethyl phthalate         | 5.0                     | 2.29                                 | 25.5                     |
| Titanium dioxide          | 0.5 (added)             |                                      |                          |

Both powders were granulated in the form of cylinders approximately 0.034 inch diameter x 0.033 inch high and then blended in the ratio of 1 part burning rate control powder to 4 parts casting powder by tumbling for 20 minutes in a sweetie barrel. The blend was transferred to a wooden hopper from which 3,540 g. was discharged through an 0.75-inch opening directly into a transparent plastic cylindrical mold 4 inches inside diameter and 18 inches long. The mold was vibrated by an air-operated vibrator (frequency 3,000 vibrations per minute, ampli-

tude 0.03 inch) for about 1 minute in order to compact the powder.

The powder-filled mold was then examined to determine homogeneity. Since the titanium dioxide colored the casting powder granules white and the carbon black colored the burning rate control powder granules black, any lack of uniformity in the distribution of the black granules through the white granules was clearly evident. When faulty distribution was detected, the contents of the mold were dumped back into the sweetie barrel for reblending and the mold refilled. Six molds were emptied and refilled in preparing the samples of twenty-one castings. Although some of the charges reblended might have burned entirely satisfactory in combustion tests, it is significant that the operator was dissatisfied with the degree of uniformity in the distribution of the black and white granules.

The mold was evacuated for 1 hour at a pressure of 4 mm. mercury to remove surface moisture from the powder, a 20-pound weight placed on top of the powder column, and 1,610 g. of casting solvent or plasticizer mixture, which had been previously evacuated for 3 hours at a pressure of 3 mm. mercury to remove moisture and dissolved air, admitted into the mold through 0.375 inch diameter tube at the rate of 270 g. per minute. When the liquid had displaced the air in the powder column and formed a layer about 0.1 inch above the column, the flow of plasticizer was stopped, the tube in the bottom of the mold closed off and disconnected from the plasticizer reservoir, and the weight removed from the top of the column. The casting was cured for 40 hours at 60° C.

All castings were satisfactory in static burning tests at normal temperature. Pressures were very uniform throughout each test.

In the preparation of cast propellants in accordance with this invention, the powder components, including the plasticizers, if desired, are given distinctively different colors. This may be accomplished in any suitable manner and at any point in the process prior to mixing and introducing the powders into the casting container. Preferably, the powder components are colored by adding the desired tinting agent to the powder ingredients during mixing or colloidizing. Alternatively, the color may be added as a surface coating after the granules have been dried. Other means will suggest themselves and are contemplated as being within the scope of the invention.

The coloring ingredients may comprise any suitable materials which impart distinctive colors such as black, white, red, yellow, green, etc., to the powder components. Thus, dyestuffs or inorganic pigments such as iron oxide, lead chromate, chromium oxide, titanium oxide, and zinc oxide or organic pigments such as para red, yellow lakes and phospho-tungstic greens are typical examples of suitable materials which can be used. In addition, many of the organic dyestuffs and other similar coloring agents may be used. Where it is desirable to incorporate an opaquing agent in large-web propellents to prevent "worm holing" during combustion, the presence of such material need not interfere with coloring of the granules, for it is possible to select opaquing agents that in themselves impart the desired contrast to the powder granules. Such a selection is illustrated by the example, where titanium dioxide was used in the casting powder and carbon black was used in the burning rate control powder.

The coloring ingredient is added in comparatively minor amounts so as not to substantially detract from the calorific value of the powder. Thus, from about 0.4% to about 0.6% by weight of the powder component has been found to give good results and is preferred. Such amounts are not critical, however, and may be varied in accordance with particular desires and usages as long as the desired distinctive color characteristics are imparted to the powder.

Inspection for nonuniformity may be made at any point in the operation after the powder has been added to the mold. However, the chances of detecting faulty grains and reusing the smokeless powder components are greatest before the casting solvent has been added to the mold and hence it is preferred to make the principal inspection at this time. Alternate or additional inspections may be made after the casting solvent has been added and/or after the casting has been cured.

Inspection of the casting may be made in any suitable manner and with any suitable means by which nonuniformity in distribution of the powder components may be determined. Since the naked eye is very sensitive to faulty patterns, visual inspection is entirely adequate and is preferred. However, it is within the scope of this invention to use such devices as photoelectric cells, or photometers specially adapted to indicate when the distribution of the powder components is faulty.

The powder components in accordance with this invention will comprise a granular casting powder, a burning rate control powder in the form of granules, strands or filaments, and a casting solvent consisting essentially of a mixture of nonvolatile plasticizers. Composition and formulation of the powder components may be as set forth in the example or in accordance with principles well known in the art. As pointed out hereinbefore, the coloring agent may be added during mixing of the ingredients of the powder components or after the powder components have been prepared.

The granular casting powder and burning rate control powder are mixed or blended in any suitable manner such as, for example, in a sweetie barrel and introduced at an even rate into the casting container. If the burning rate control powder is in the form of strands or filaments, these are anchored in spaced relation by upper and lower perforated discs, placed in the casting container, and casting powder poured in around them. A weighted member is then placed on the powder column to hold the granules in place during subsequent operations.

The casting container is formed of a nonflammable, transparent material to inhibit burning of the cast propellant and to permit inspection of the powder components after they have been introduced into the container. Preferred materials of this type are those which can be plasticized by the casting solvents, so as to secure a strong bond between the powder and container. An example of such preferred material is cellulose acetate.

The nonvolatile plasticizers or casting solvent are preferably admitted to the container or mold through an opening in its bottom portion and forced upwardly through the powder column under a pressure head created by raising the liquid level of the plasticizer several feet above the top of the mold. Any other means such as pumps, reduced pressure inside the mold, etc., could be used provided the introduction of the liquid is accomplished at the desired steady rate. The rate at which the plasticizer rises in the mold will desirably be as great as possible without entrapping air in the powder column. Upward displacements varying from about 5 to about 10 inches per minute are preferred, although rates as high as 20 inches per minute may be used especially with larger powder granules and less viscous plasticizers than those cited in the example. The opening for admitting the plasticizer may be of any suitable size and is located in any portion of the bottom of the mold. Preferably, the size of the opening will be from about  $\frac{1}{8}$  inch to about 1 inch and centrally located.

After the plasticizer has been introduced, the weight on top of the powder column is removed and the container with contents placed in a heated atmosphere to cure. Curing is desirably accomplished by placing the casting in a forced air oven for a period from about 1 hour to about 600 hours and at a temperature from about 30° C. to about 80° C., and preferably for about 40 hours at 60° C. It will be realized, of course, that any suitable

type of drying and/or curing device may be used and that temperatures and times may be adjusted and coordinated by principles well known in the art.

The device of the present invention can be used in any composite smokeless powder charge or load, in which the arrangement or distribution of the component powder particles must follow a prearranged order. It has widest application to the manufacture of cast propellants for use in rockets, assisted takeoff motors, and other jet-controlled uses.

The present invention provides a quick, easy, and inexpensive way to insure that the powder components are properly arranged through the casting. By inspecting the castings just before the plasticizers are added, it is possible to recover and reuse the powder and plastic mold components of faulty castings, simply by pouring the powder back into the blending barrels, and refilling the molds. Finished castings may likewise be examined and faulty distribution detected. As a result, faulty castings giving irregular burning with consequent hazards and undependability in use, are eliminated.

What I claim and desire to protect by Letters Patent is:

1. In the manufacture of cast smokeless powder propellents from a mixture of powder ingredients, the method which comprises forming the powder components with distinctly different colors, mixing the powder components so as to obtain a uniform color pattern indicative of the homogeneity of the powder, introducing a mixture into a transparent container to form a charge, introducing a casting solvent through an opening in the bottom of said transparent container and curing the contents of said container at an elevated temperature to form a casting.

2. A method in accordance with claim 1 in which the distinctly different colors are obtained by the addition of coloring agents to the powder components during formulation thereof.

3. A method in accordance with claim 1 in which the distinctly different colors are obtained by the addition of coloring agents to the powder components after formulation thereof.

4. A method in accordance with claim 1 in which the distinctly different colors are obtained by coating the powder components.

5. A method in accordance with claim 1 in which the distinctly different colors are obtained by the addition of inorganic pigments to the powder components.

6. A method in accordance with claim 1 in which the distinctly different colors are obtained by the addition of organic pigments to the powder components.

7. In the manufacture of cast smokeless powder propellents from powder components including a casting powder, a burning rate powder and a casting solvent, the method which comprises forming the powder components with distinctly different colors, mixing the casting powder and the burning rate control powder so as to obtain a uniform color pattern indicative of the homogeneity of the powder, introducing the mixture into a transparent container to form a charge, introducing a casting solvent

through an opening in the bottom of said transparent container and curing the contents of said container at an elevated temperature to form a casting.

8. In the manufacture of cast smokeless powder propellents from a mixture of powder components and a casting solvent, the method which comprises coloring the powder components with coloring agents producing distinctly different colors, at least one of said coloring agents being titanium dioxide, mixing the powder components so as to obtain a uniform color pattern indicative of the homogeneity of the powder, introducing the mixture into a transparent container to form a charge, introducing the casting solvent through an opening in the bottom of said transparent container and curing the contents of said container at an elevated temperature to form a casting.

9. In the manufacture of cast smokeless powder propellents from a mixture of powder components and a casting solvent the method which comprises coloring the powder components with coloring agents producing distinctly different colors, at least one of said coloring agents being carbon black, mixing the powder components so as to obtain a uniform color pattern indicative of the homogeneity of the powder, introducing the mixture into a transparent container to form a charge, introducing the casting solvent through an opening in the bottom of said transparent container and curing the contents of said container at an elevated temperature to form a casting.

10. In the manufacture of cast smokeless powder propellents from a mixture of powder components and a casting solvent the method which comprises coloring the powder components with coloring agents producing distinctly different colors, at least one of said coloring agents being para red, mixing the powder components so as to obtain a uniform color pattern indicative of the homogeneity of the powder, introducing the mixture into a transparent container to form a charge, introducing the casting solvent through an opening in the bottom of said transparent container and curing the contents of said container at an elevated temperature to form a casting.

30

35

40

#### References Cited by the Examiner

##### UNITED STATES PATENTS

|           |         |             |          |
|-----------|---------|-------------|----------|
| 1,605,655 | 11/1926 | Du Pont     | 102—42   |
| 2,353,934 | 7/1934  | Schreib     | 102—38   |
| 2,417,090 | 3/1947  | Silk et al. | 52—0.5 X |
| 2,440,327 | 4/1948  | Crawford.   |          |
| 2,574,479 | 11/1951 | Hickman.    |          |
| 2,643,611 | 6/1953  | Ball        | 52—0.5 X |

##### FOREIGN PATENTS

21,240 1906 Great Britain.

LEON D. ROSDOL, *Primary Examiner.*

ALEXANDER BISHOFF, WILLIAM G. WILES,  
55 ROGER L. CAMPBELL, *Examiners.*

L. H. MYERS, A. P. KENT, W. A. KEMMEL,  
Assistant Examiners.